

## UNITED STATES PATENT OFFICE

1,934,414

GRAINED WOOD AND METHOD OF  
GRAINING SAME

Charles Joseph Fess, Maplewood, N. J.

No Drawing. Application March 4, 1931  
Serial No. 520,158

2 Claims. (Cl. 41—41)

This invention relates to the artificial graining of wood and has for its principal objects the simple, expeditious and economical reproduction upon various woods of an accurate and faithful simulation of the grain of another wood whereby the selected woods can be profitably employed in the production of furniture, pianos, trim and cabinet work and all of the advantages possessed by another wood, the grain of which has been simulated, are obtained and, in addition thereto, the advantages possessed by the selected wood, such as its ability to resist warping, its low cost, the reduction in wastage caused in matching up the grain and the like are retained, while at the same time the disadvantages of a poor appearance, due either to the fact of the substantial absence of grain or the fact that the natural grain thereof is unattractive or undesirable, is avoided.

I am aware that it has been proposed to utilize, either in the graining of wood or metal, a negative comprising a natural wood panel whose grain corresponds to that of the wood, the grain of which it is desired to imitate, and also that it has been proposed to apply to a wood or metal panel to be grained and opaque coat containing a solid pigment or color corresponding to the base or ground color desired in the finished panel. However, no one so far, as I am aware, has been able to reproduce on a selected wood such a perfect and accurate simulation of the grain of another wood as is accomplished by the method hereinafter described.

In carrying out my invention, I preferably proceed as follows:—

35 The wood panel or wood article to be grained, such for example, as a panel of maple, is prepared as follows:—

1. The panel is first planed, scraped and smoothed to an even flat surface and is then stained with a soluble stain, such for example as an aniline color dissolved in water, alcohol or oil, which stain is of such a color that its effect after application to the article is to make the latter's general color tone match the base color 40 of the wood which it is intended to simulate. After such stained surface is dry, a thin coat of shellac or other generally used sealer is then applied to the stained surface in order not only to enhance or intensify the appearance of the 45 stain so applied but also, to produce after the staining thereof, a level surface in order to insure perfect contact between the surface and the roller in the transfer process hereinafter described.

55 2. To prepare said graining plate, a panel of

the natural wood, whose grain it is desired to simulate, is first planed, scraped and smoothed to an even flat surface. The surface of the wood is then saturated with a 10% aqueous solution of borax heated to about 100° C. While the wood 60 is still wet, it is brushed with a stiff bristle or fibre brush, the surface being scrubbed against the grain, and the bristles worked well into the pores. The surface is then rinsed thoroughly with water, allowed to dry and is finely sanded 65 with sandpaper, whereupon a coat of pyroxylin lacquer is applied to such smooth sanded surface to seal the same and prevent penetration of the graining ink into the pores.

3. After the lacquer coat has dried, the said 70 graining plate is first completely coated with a graining ink, the surplus ink is scraped off with a doctor blade in the well known manner and then a soft elastic roller, known as a transfer roller, is then first rolled over such plate whereby the inked 75 graining pattern thereon is transferred to the peripheral surface of the roller.

The graining pattern picked up by the soft transfer roll is then immediately transferred in the well known manner to the prepared surface 80 of the wood to be grained, the same being accomplished by a single pass of the roll over such surface, while applying to such roll sufficient pressure to effect intimate contact between the engaging surfaces and to thereby obtain a substantially complete transfer of the ink from the grain portions of the plate to the receptive surface 85 of the wood to be grained.

The employment of a soluble and transparent coloring medium in the stain applied to the surface to be grained is an essential feature of the preparation of the wood for the reception of the graining pattern. Not only does this transparent stain accomplish the substantial masking or camouflaging of the natural grain of such wood so selected, but at the same time I preserve, substantially unimpaired, the softness and brilliancy of depth of natural wood and the original tonal effect or light reflection and refraction from natural grain of the wood employed, such for 90 example as maple, birch, plain sawed oak and the like, selected for the graining operation and as a consequence, the ultimate effect obtained is, unlike that obtained heretofore, distinguished with difficulty from a finished surface of the natural 95 wood which has been imitated.

While I prefer to apply a thin coat of pyroxylin lacquer to the wood graining plate as aforesaid because of the fact that, owing to its toughness and elasticity, even an extremely thin coat there- 100 105 110

of serves to offer permanent resistance to penetration of the graining inks applied to such plate into the pores of the walls of the ink receptacles thereof and, owing to the thinness of the film required, such film does not obscure or clog the ink-receiving cells of the graining plate.

Altho I preferably employ a 10% solution of borax heated to a boiling temperature for the treatment of the panel selected for the graining plate, borax solutions of other concentrations, such for example as a 5% concentration or even concentrations greater than 10% may be employed and the time of treatment would be varied accordingly. The borax is employed because this substance, unlike strong alkalies, such as caustic soda, for example, does not tend to destroy or even substantially swell the wood fibres in the hard grain areas, while at the same time, it assists, as heretofore explained, in the elimination by the brushing operation of the pulp and pulp areas, as well as the fibres overlying such areas. The principal advantage of the use of borax is that it does not destroy or make ragged the edges of the areas surrounding or constituting the walls of the pores, which, as above stated, is in contrast to the action of strong or so-called caustic alkalies.

The shellac or like sealing coat, which is applied to seal the surface of the wood selected to be grained, is sanded or otherwise treated after such coat has dried in order to remove the glossy appearance and afford a receptive surface that will insure intimate union with the graining ink subsequently applied thereto by means of the transfer roller. Preferably, also, the stain employed is a water stain containing a water-soluble dye or coloring medium as such stain will, when a subsequent sealing coat of shellac in alcohol is applied thereto, tend to enhance or intensify the coloring effect of the stain so applied.

Among the essential advantages obtained through the employment of my improved graining method are that it is possible to change the ground color and obscure or mask the natural grain of the wood to be artificially grained, without however, obscuring or losing the natural tonal effect or inimitable "wood" appearance of depth and softness imparted thereby and upon this enhanced background to impose the more

beautiful grain of the wood whose grain it is desired to imitate.

While I preferably employ the herein described wood graining plate for effecting the transfer of the desired grain to the surface prepared to receive the same, other graining plates, such as intaglio metal graining plates, whereon the graining pattern has been photographically reproduced, can be substituted therefor. Also various other changes within the scope of the appended claims may be made without departing from the spirit of my invention as herein set forth.

Having thus described my invention, what I claim and desire to obtain by United States Letters Patent is:—

1. The method of making a graining plate for reproducing the grain of wood on a solid surface which comprises providing a smooth, even surface on the piece of wood selected for such plate, subjecting the surface of the wood to the action of a hot concentrated aqueous solution of an alkaline sodium compound containing the boric acid radical in its composition and while still wet subjecting the same to an abrasive and effecting the removal of the cellular material from the pores of the wood so as to provide ink receptacles, then rinsing said surface to thoroughly remove the alkaline solution, drying the surface, smoothing such surface with fine abrasive material and then sealing the exposed portions of the surface of the wood with a thin water-proofing protective coating to prevent penetration of ink into the pores of such surface.

2. The process of making a graining plate, which comprises subjecting the surface of a specimen of wood, the grain of which it is desired to reproduce, to the action of a concentrated solution of borax, while heated substantially to a boiling temperature, in order to render the pulp readily removable, then while the surface is still wet, subjecting the pulp containing areas to an abrasive element to remove the contained pulp and overlying fibers from such areas, then rinsing the surface to remove the aforesaid borax solution, drying the same, again smoothing said surface to remove projecting fibers and then applying a thin coat of pyroxylin lacquer to such surface portions of the wood specimen so treated.

CHARLES JOSEPH FESS.

50

55

60

65

70

75

80

85

90

95

100

105

110

115

120

125

130

135

140

145

150